

## 1

2,709,129

## IGNITER COMPOSITIONS

Franklin B. Clay, Westport, and Richard A. Sahlin, Fairfield, Conn., assignors to Remington Arms Company, Inc., Bridgeport, Conn., a corporation of Delaware

No Drawing. Application December 31, 1952,  
Serial No. 329,111

2 Claims. (Cl. 52—2)

This invention relates to igniter compositions for tracer projectiles, and contemplates an igniter that will burn and perform its function of igniting the actual tracer composition with little if any flame or light.

Tracer projectiles are particularly useful for the firing of aircraft guns and perform the function of indicating the direction of fire of a gun on a somewhat unstable mount with respect to a target usually having a high speed of movement relative to the gun. It is essential that the trace be clearly visible to the gunner or observer in the region of the target, but the flash of light immediately adjacent the muzzle of the gun has an adverse effect on the shooter's vision and his ability to accurately observe the trace in the region where the trace is of significance.

The present invention contemplates an igniter composition which leaves an invisible or dim trace to a minimum distance of twenty-five (25) yards and a bright and properly colored trace at greater distances.

Conventional igniter compositions comprise a very active fuel, such as powdered magnesium, tempered with a less energetic fuel, such as calcium resinate, and an active oxidizer and coloring agent which may be an admixture of such reagents as the peroxides of barium, strontium and lead. Igniters of this type burn immediately with a very luminous flame with an undesirable blinding of the observer by the bright trace at the short ranges where the trace is of little if any value.

It has been found that igniter compositions which include a fuel of the type of calcium silicide, as a partial or entire replacement for a fuel of the type of magnesium, burn in such a manner that the trace for a minimum distance of twenty-five (25) yards is only dimly visible if visible at all. Notwithstanding this, these compositions effectively perform their intended function of igniting the actual tracer composition at a range of twenty-five (25) to seventy-five (75) yards, the com-

## 2

bustion of the tracer composition thereafter furnishing a trace of the desired color, intensity and duration.

Typical igniter compositions according to the invention are as follows:

| 5  |                         | Range, Percent | Preferred, Percent |
|----|-------------------------|----------------|--------------------|
|    | Strontium Peroxide..... | 75.0-81.0      | 78                 |
| 10 | Barium Peroxide.....    | 3.9- 4.1       | 4                  |
|    | Lead Peroxide.....      | 3.9- 4.1       | 4                  |
|    | Calcium Resinate.....   | 6.0- 8.0       | 7                  |
|    | Calcium Silicide.....   | 3.0-11.0       | 7                  |

As compared with compositions containing magnesium or like fuel, the compositions of this invention show materially improved stability in storage; cartridges containing them, after storage periods of up to sixty-seven (67) weeks, showed only a small fraction of the failures to ignite and other defects exhibited by cartridges loaded with magnesium-containing igniters stored under identical conditions.

What is claimed is:

1. An igniter for tracer compositions consisting essentially of—

| 25 |                         | Per cent  |
|----|-------------------------|-----------|
|    | Strontium peroxide..... | 75.0-81.0 |
|    | Barium peroxide.....    | 3.9- 4.1  |
|    | Lead peroxide.....      | 3.9- 4.1  |
|    | Calcium resinate.....   | 6.0- 8.0  |
| 30 | Calcium silicide.....   | 3.0-11.0  |

2. An igniter for tracer compositions consisting essentially of—

| 35 |                         | Per cent |
|----|-------------------------|----------|
|    | Strontium peroxide..... | 78       |
|    | Barium peroxide.....    | 4        |
|    | Lead Peroxide.....      | 4        |
|    | Calcium resinate.....   | 7        |
|    | Calcium silicide.....   | 7        |

## References Cited in the file of this patent

## UNITED STATES PATENTS

|           |           |               |
|-----------|-----------|---------------|
| 1,708,187 | Meek      | Apr. 9, 1929  |
| 1,756,255 | Meek      | Apr. 29, 1930 |
| 1,903,814 | Graff     | Apr. 18, 1933 |
| 2,115,047 | Stevenson | Apr. 26, 1938 |
| 2,115,608 | Brandt    | Apr. 26, 1938 |
| 2,410,801 | Audieth   | Nov. 12, 1946 |

## FOREIGN PATENTS

|    |         |               |              |
|----|---------|---------------|--------------|
| 50 | 275,021 | Great Britain | Aug. 4, 1927 |
|----|---------|---------------|--------------|